# EUROPEAN PATENT SPECIFICATION

(11) **EP 1 585 852 B1**
(45) Date of publication and mention of the grant of the patent: **04.02.2009**
(21) Application number: 03782261.6
(22) Date of filing: 01.12.2003
(51) Int. Cl.: D03D 15/00, D04H 13/00

(54) **FABRIC WITH A BASE OF NON-WOVEN FABRIC STRIPS**
GEWEBE AUF BASIS VON BÄNDERN AUS VLIESSTOFF
STRUCTURE TEXTILE COMPORTANT UNE BASE DE BANDES TEXTILES NON TISSÉES

(30) Priority: 06.12.2002 IT MI20022595
(43) Date of publication of application: 19.10.2005
(73) Proprietor: Orlandi S.p.A., 20122 Milano (IT)
(72) Inventor: ORLANDI, Vittorio, I-21010 Arsago Seprio (IT)
(74) Representative: Gerli, Paolo
(86) International application number: PCT/EP2003/013503
(87) International publication number: WO 2004/053216

(56) References cited:
- EP-A- 0 277 668
- EP-A- 0 678 607
- WO-A-98/46817
- DE-A- 3 437 202
- US-A- 1 829 299
- US-A- 2 106 457

## Description

### FIELD OF THE INVENTION

The present invention concerns the field of articles in non-woven fabric, with particular application in the field of cleaning and/or protection of surfaces in the home.

### PRIOR ART

Materials with a non-woven base are widely applied in various sectors. In the procedures for producing articles with a non-woven base, this product is normally unwound from bobbins which hold it and processed by means of the treatments required by the article concerned (for example stitching, rolling, incision of patterns in relief, moulding, cutting into the final shape, etc.); collateral with these procedures it the production of high quantities of waste non-woven fabric, composed of the trimmings left over from cutting the fabric into the desired dimensions and shape. Most of these trimmings are in the form of strips of various length, derived from lengthwise cutting of the peripheral portions of non-woven fabric unwound from the bobbin.

These materials are normally discarded or recycled in the production of low-value products. The products of recycling thus obtained do not cover the value of the original material lost in the waste: it is therefore desirable to reduce the waste of material in these procedures, or to increase the economic yield of the recycling of waste, so as to reduce the overall cost of the procedures for producing articles in non-woven fabric.

EP 277 668 generically refers of fibrous web materials; in one embodiment, a fabric composed of weft and warp is shown, wherein the composing strips are made of needled fibrous material.

### SUMMARY

The present invention allows to increase the economic yield of the recycling of waste from the processing of non-woven fabric. This result has been obtained by applying the techniques of weaving to non-woven fabrics, that is those materials which on account of their nature do not require any weaving.

Using this method it has been possible to obtain textile products composed of strips of non-woven fabric interwoven like weft and warp. The products thus obtained, intended for the cleaning and protection of various surfaces, for example in the home, have performances equal to or superior to those of traditional products with a base of textile fibres.

### DETAILED DESCRIPTION OF THE INVENTION

The object of the present invention is a textile product composed of a weft and a warp, in which the weft and the warp are composed of strips of non-woven fabric.

It has in fact been observed that strips of non-woven fabric, such as those obtained from production trimmings, can be used in the same way as textile products on a loom and interwoven in the form of a weft and warp, thus obtaining a fabric with a base of non-woven fibres.

The resulting textile product has proved to be a high-strength product with considerable versatility of application: in particular the best application of the fabric is in the field of cleaning or protection of various surfaces. It can therefore be used in the manufacture of cloths for cleaning floors, of cloths for cleaning small surfaces in the home (e.g. bathroom, kitchen, etc.), tablecloths, napkins, matting, mats, bedspreads, couch covers, cushion covers, car seat covers, doormats.

All the manufactures obtained with the textile product concerned are also part of the present invention.

The strips of non-woven fabric used in the present invention are composed of hydroentangled fibres. Examples of materials that constitute non-woven fibres are: viscose, polyethylene, polypropylene, polyamide, cellulose pulp.

For the above applications in the field of cleaning and protecting surfaces, the non-woven fabric used has a weight/surface ratio between 10 g/m² and 200 g/m², preferably between 50 g/m² and 65 g/m².

In the invention, both the weft and the warp of the textile product concerned are composed of strips of non-woven fabric: this process results in products with considerable uniformity.

The strips of which the present textile product are made have a width generally between 1 and 10 cm, preferably between 4 and 7 cm.

As indicated above, the non-woven strips may be a sub-product obtained from processing waste, typically represented by strips of trimmings of non-woven fabric unwound from bobbins or reels. This method is therefore excellent for recycling these materials, obtaining a material with high added value and thus fully recovering the value of the material discarded during the processes for the production of articles in non-woven fabric.

Although this invention is advantageously suitable for the recovery of processing trimmings, it is nevertheless not to be understood as limited to the use of that raw material. It is in fact also possible, and is part of the present invention, to realise made-do-measure strips having the desired shape, dimensions and weight, and to interweave them together in the form of a weft and warp, in order to obtain products with particular characteristics. It is clear that in this case, thanks to the constant and controlled dimensions of the strips used, the product will present greater uniformity and constancy of characteristics in comparison with a product obtained from recycling strips, which are generally more variable in shape, dimensions and weight.

In a non limiting example of an embodiment of the present invention, selvedges (trimmings) of 4-5 cm were used, with a weight of 50-55 g/cm²; the selvedges were fed into a loom for weaving special products (with high teething), at the speed of 1 m/h, obtaining a web with a height of 160 cm and a roll with a diameter of 50 cm; cloths were made with dimensions 40 cm X 50 cm with absorbent capacities equivalent to those of products (polyester viscose) used on the market.

The strength in both CD *(cross direction)* and MD *(machine direction)* was considerably increased (about 3 times that of standard products). The cloth presented considerable duration and resistance in time after being used to clean floors.

## Claims

1. Textile product composed of a weft and a warp, in which the weft and the warp are composed of strips of non-woven fabric, **characterised in that** the non-woven fabric is composed of hydroentangled fibres.

2. Textile product according to claim 1, wherein the non-woven fabric is composed of a material chosen from viscose, polyethylene, polypropylene, polyamide, cellulose pulp.

3. Textile product according to claims 1-2, wherein the non-woven fabric has a weight/surface ratio between 10 g/m² and 200 g/m².

4. Textile product according to claim 3, wherein the non-woven fabric has a weight/surface ratio of between 50 g/m² and 65 g/m².

5. Textile product according to claims 1-4, wherein said strips of non-woven fabric have a width between 1 and 10 cm.

6. Textile product according to claim 5, wherein said strips of non-woven fabric have a width between 4 cm and 7 cm.

7. Textile product according to claims 1-6, wherein said strips of non-woven fabric are obtained from processing waste.

8. Procedure for the preparation of the textile product described in claims 1-7, **characterised in that** the strips of non-woven fabric are subjected to weaving, realising a fabric in which the weft and the warp are composed of said strips of non-woven fabric.

9. Manufacture realised with the textile product described in claims 1-7.

## Patentansprüche

1. Textiles Erzeugnis, bestehend aus Schuss und Kette, bei welchem Schuss und Kette aus Streifen aus Faservliesmaterial bestehen, **dadurch gekennzeichnet, dass** das Faservliesmaterial aus hydraulisch verwirbelten Fasern besteht.

2. Textiles Erzeugnis nach Anspruch 1, bei welchem das Faservliesmaterial aus einem der Materialien besteht, zu denen Viskose, Polyethylen, Polypropylen, Polyamid, Zellulosebrei gehören.

3. Textiles Erzeugnis nach Anspruch 2, bei welchem das Faservliesmaterial ein Flächengewicht zwischen 10 g/m² und 200 g/m² aufweist.

4. Textiles Erzeugnis nach Anspruch 3, bei welchem das Faservliesmaterial ein Flächengewicht zwischen 50 g/m² und 65 g/m² aufweist.

5. Textiles Erzeugnis nach Anspruch 1 - 4, bei welchem die genannten Streifen des Faservliesmaterials eine Breite zwischen 1 und 10 cm aufweisen.

6. Textiles Erzeugnis nach Anspruch 5, bei welchem die genannten Streifen des Faservliesmaterials eine Breite zwischen 4 und 7 cm aufweisen.

7. Textiles Erzeugnis nach Anspruch 1 - 6, bei welchem die genannten Streifen des Faservliesmaterials aus der Verarbeitung von Abfall erhalten werden.

8. Verfahren zur Herstellung des in den Ansprüchen 1 - 7 beschriebenen textilen Erzeugnisses, **dadurch gekennzeichnet, dass** die Streifen aus Faservliesmaterial dem Webvorgang unterzogen werden, wodurch ein Stoff entsteht, bei welchem Schuss und Kette aus den genannten Streifen des Faservliesmaterials bestehen.

9. Fertigung unter Verwendung des in den Ansprüchen 1 - 7 beschriebenen textilen Erzeugnisses.

## Revendications

1. Produit textile constitué d'une chaîne et d'une trame, où la chaîne et la trame sont constituées de bandes de tissu non-tissées, **caractérisé en ce que** le tissu non-tissé est constitué de fibres hydro-enchevêtrées.

2. Produit textile selon la revendication 1, où le tissu non-tissé est constitué d'un matériau sélectionné parmi la viscose, polyéthylène, polypropylène, polyamide, pâte cellulosique.

3. Produit textile selon les revendications 1-2, où le tissu non-tissé présente un rapport de poids/surface entre 10 g/m² et 200 g/m².

4. Produit textile selon la revendication 3, où le tissu non-tissé présente un rapport de poids/surface entre 50 g/m² et 65 g/m².

5. Produit textile selon les revendications 1-4, où lesdites bandes du tissu non-tissé ont une largeur entre 1 et 10 cm.

6. Produit textile selon la revendication 5, où lesdites bandes de tissu non-tissé ont une largeur entre 4 cm et 7 cm.

7. Produit textile selon les revendications 1-6, où lesdites bandes de tissu non-tissé sont obtenues par le traitement de déchets.

8. Procédé de préparation du produit textile décrit dans les revendications 1-7, **caractérisé en ce que** les bandes de tissu non-tissé sont soumises au tissage, en réalisant un tissu dans lequel la trame et la chaîne sont constituées desdites bandes de tissu non-tissé.

9. Article manufacturé réalisé avec le produit textile décrit dans les revendications 1 à 7.
